



US011331939B2

(12) **United States Patent**  
**Zhou et al.**

(10) **Patent No.:** **US 11,331,939 B2**  
(45) **Date of Patent:** **May 17, 2022**

(54) **RECORDING MEDIA**

(71) **Applicant:** **HEWLETT-PACKARD DEVELOPMENT COMPANY, L.P.**,  
Spring, TX (US)

(72) **Inventors:** **Xiaoqi Zhou**, San Diego, CA (US);  
**David Edmondson**, San Diego, CA (US); **Rodney D. Stramel**, San Diego, CA (US)

(73) **Assignee:** **Hewlett-Packard Development Company, L.P.**, Spring, TX (US)

(\*) **Notice:** Subject to any disclaimer, the term of this patent is extended or adjusted under 35 U.S.C. 154(b) by 188 days.

(21) **Appl. No.:** **16/705,970**

(22) **Filed:** **Dec. 6, 2019**

(65) **Prior Publication Data**

US 2020/0180338 A1 Jun. 11, 2020

**Related U.S. Application Data**

(63) Continuation of application No. 14/113,567, filed as application No. PCT/US2011/034400 on Apr. 28, 2011, now Pat. No. 10,543,707.

(51) **Int. Cl.**

**B41M 5/00** (2006.01)  
**B41M 5/50** (2006.01)  
**B41M 5/52** (2006.01)

(52) **U.S. Cl.**

CPC ..... **B41M 5/0017** (2013.01); **B41M 5/506** (2013.01); **B41M 5/52** (2013.01); **B41M 5/5254** (2013.01); **Y10T 428/24802** (2015.01)

(58) **Field of Classification Search**

CPC .. **B41M 5/0017**; **B41M 5/5254**; **B41M 5/506**; **B41M 5/52**

USPC ..... 428/195.1  
See application file for complete search history.

(56)

**References Cited**

## U.S. PATENT DOCUMENTS

|             |         |                   |
|-------------|---------|-------------------|
| 4,328,284 A | 5/1982  | LePoutre          |
| 4,489,188 A | 12/1984 | Jones et al.      |
| 5,236,987 A | 8/1993  | Arendt            |
| 5,308,680 A | 5/1994  | Desjarlais et al. |

(Continued)

## FOREIGN PATENT DOCUMENTS

|    |             |        |
|----|-------------|--------|
| CN | 1352599 A   | 6/2002 |
| CN | 101365760 A | 2/2009 |

(Continued)

## OTHER PUBLICATIONS

BASF, Acronal S 782 na, Feb. 2015, p. 1, retrieved from [https://worldaccount.bASF.com/wa/NAFTA-en\\_US/Catalog/Additives/doc/BASF/PRD/30193826.pdf?asset\\_type=pi/pdf&language=EN&urn=urn:documentumCommerce\\_sol\\_EU:09007bb280178723.pdf](https://worldaccount.bASF.com/wa/NAFTA-en_US/Catalog/Additives/doc/BASF/PRD/30193826.pdf?asset_type=pi/pdf&language=EN&urn=urn:documentumCommerce_sol_EU:09007bb280178723.pdf) (Year: 2015).

(Continued)

*Primary Examiner* — Betelhem Shewareged

(74) **Attorney, Agent, or Firm:** HP Inc. Patent Department

(57)

**ABSTRACT**

A recording media containing a raw base substrate having, on its image side, a primary coating layer and a top image receiving layer is described herein. Said top image receiving layer encompasses a polymeric adhesion promoter having a glass transition temperature that is at, or above, 90° C. Also described is a printed article containing said recording media on which a printed feature has been formed with an ink composition that encompasses latex components that have a glass transition temperature that is at, or above, 90° C.

**18 Claims, 2 Drawing Sheets**

(56)

**References Cited**

## U.S. PATENT DOCUMENTS

|                  |         |                   |            |               |             |         |
|------------------|---------|-------------------|------------|---------------|-------------|---------|
| 6,248,432 B1     | 6/2001  | Moronuki et al.   | EP         | 2050784 A1    | 4/2009      |         |
| 6,372,329 B1     | 4/2002  | Graczyk et al.    | JP         | 2000-007961   | 1/2000      |         |
| 6,447,883 B1     | 9/2002  | Chen et al.       | JP         | 2005-048014   | 2/2005      |         |
| 6,506,479 B1     | 1/2003  | Horiuchi          | JP         | 2005-062845   | 3/2005      |         |
| 7,696,262 B2     | 4/2010  | Cagle et al.      | JP         | 2006-103194   | 4/2006      |         |
| 7,754,296 B2     | 7/2010  | Khoutchaev et al. | JP         | 2006-110986   | 4/2006      |         |
| 7,811,656 B2     | 10/2010 | Grandhee et al.   | JP         | 2006-240257   | 9/2006      |         |
| 2004/0115557 A1  | 6/2004  | Bourdelaix et al. | JP         | 2007-290339   | 11/2007     |         |
| 2005/0191445 A1  | 9/2005  | Sen et al.        | JP         | 2008-207409   | 9/2008      |         |
| 2006/0205840 A1* | 9/2006  | Kato .....        | C09D 11/40 | JP            | 2008-246946 | 10/2008 |
|                  |         |                   | 523/160    | JP            | 2009-113292 | 5/2009  |
| 2007/0218254 A1  | 9/2007  | Zhou et al.       | JP         | 2010-094850   | 4/2010      |         |
| 2007/0242124 A1  | 10/2007 | Tomita et al.     | JP         | 2010-162759   | 7/2010      |         |
| 2008/0057230 A1  | 3/2008  | Read et al.       | JP         | 2011-042150   | 3/2011      |         |
| 2008/0081134 A1  | 4/2008  | Irita et al.      | WO         | WO-2003078513 | 9/2003      |         |
| 2008/0233352 A1  | 9/2008  | Smith et al.      | WO         | WO-2007095136 | 8/2007      |         |
| 2010/0243141 A1  | 9/2010  | Muro et al.       |            |               |             |         |
| 2011/0030709 A1* | 2/2011  | Sebastian .....   | A24C 5/34  |               |             |         |
|                  |         |                   | 131/365    |               |             |         |
| 2013/0201251 A1  | 8/2013  | Pal et al.        |            |               |             |         |
| 2020/0180338 A1* | 6/2020  | Zhou .....        | B41M 5/52  |               |             |         |

## FOREIGN PATENT DOCUMENTS

|    |             |        |
|----|-------------|--------|
| CN | 101668629 A | 3/2010 |
| EP | 1232873 A1  | 8/2002 |

## OTHER PUBLICATIONS

Petri et al, High performance Acrylic Dispersions for Masonry and Wood Coatings, Nov. 5, 2015, Celanese, p. 8, retrieved from <http://www.asefapi.es/congreso3/Preview/files/CELANESE.pdf>(Year: 2015).

\* cited by examiner



**FIG. 4****FIG. 5****FIG. 6**

# 1

## RECORDING MEDIA

### CROSS-REFERENCE TO RELATED APPLICATIONS

This application is a continuation application of co-pending U.S. application Ser. No. 14/113,567, filed Oct. 23, 2013, which itself is a national stage entry under 35 U.S.C. § 371 of PCT/US2011/034400, filed Apr. 28, 2011, each of which is incorporated by reference herein in its entirety.

### BACKGROUND OF THE INVENTION

Inkjet printing technology is a non-impact printing method in which an electronic signal controls and directs droplets or a stream of ink that can be deposited on a wide variety of substrates. Inkjet technology is, nowadays, becoming a popular way of recording images on various media surfaces. Inkjet printers have thus found broad applications across markets, ranging from industrial labeling to short run printing, to desktop document, pictorial imaging and large format printing for outdoor applications such as banners, displays, posters, billboard and vehicle wraps.

It becomes apparent that the image quality and durability of printed images, obtained using such printing technology, are strongly dependent of the construction of the print media, of the ink composition used and of their interaction. Most of the inkjet ink compositions are water-based, their colorant constituents are thus often water-soluble or water dispersible. Therefore, because of their water-based nature, such inkjet inks tend to exhibit poor image durability when exposed to water or high humidity. Inkjet ink composition containing latexes have been developed in view of improving the durability of such inks. Said inks contain submicron polymeric latex particles of high molecular weight that are dispersed in an aqueous fluid. Both dyes and pigments have been used as colorants for such inkjet ink formulations. However, when the ink formulations contain latex, such materials do not always adhere well to the substrates to which the ink is applied. The resulting printed image might have durability issues such as abrasion resistance, light-fastness, solvent-fastness and water-fastness.

In inkjet printing method, the receiving media substrates play a key role in the overall image quality and permanence of the printed images. Accordingly, it has often created challenges to find media which can be effectively used with such printing techniques and which have good image quality and good adhesion capability.

### BRIEF DESCRIPTION OF THE DRAWINGS

The drawings illustrate various embodiments of the present system and method and are part of the specification.

FIG. 1, FIG. 2 and FIG. 3 are cross-sectional views of a recording media according to embodiments of the present disclosure.

FIG. 4, FIG. 5 and FIG. 6 are cross-sectional views of a printed article according to embodiments of the present disclosure.

### DETAILED DESCRIPTION

Embodiments of the present disclosure will employ, unless otherwise indicated, techniques of synthetic organic chemistry, ink chemistry, media chemistry, printing chemistry, and the like, that are within the skill of the art. Such techniques are explained fully in the literature. The

# 2

examples are put forth to provide those of ordinary skill in the art with a complete disclosure and description of how to perform the methods and use the compositions disclosed herein. Efforts have been made to ensure accuracy with respect to numbers (e.g., amounts, temperature, etc.) but some errors and deviations should be accounted for. Unless indicated otherwise, parts are parts by weight, temperature is in ° C., and pressure is at or near atmospheric. Standard temperature and pressure are defined as 20° C. and 1 atmosphere. Unless otherwise indicated, the viscosity is expressed in cP and is measured at a temperature of 25° C. Before the embodiments of the present disclosure are described in detail, it is to be understood that, unless otherwise indicated, the present disclosure is not limited to particular materials, and processes disclosed herein as such may vary to some degree. It is also to be understood that the terminology used herein is for purposes of describing particular embodiments only, and is not intended to be limiting, as the scope of the present invention will be defined only by the claims and equivalents thereof. In the present specification, and in the claims, the following terminology will be used: the singular forms “a”, “an”, and “the” include plural referents unless the context clearly dictates otherwise. Thus, for example, reference to “a support” includes a plurality of supports. The terms “about” and “approximately,” when referring to a numerical value or range is intended to encompass the values resulting from experimental error that can occur when taking measurements. Concentrations, amounts, and other numerical data may be presented herein in a range format. It is to be understood that such range format is used merely for convenience and brevity and should be interpreted flexibly to include not only the numerical values explicitly recited as the limits of the range, but also to include all the individual numerical values or sub-ranges encompassed within that range as if each numerical value and sub-range is explicitly recited. For example, a weight range of approximately 1 wt % to approximately 20 wt % should be interpreted to include not only the explicitly recited concentration limits of 1 wt % to approximately 20 wt %, but also to include individual concentrations such as 2 wt %, 3 wt %, 4 wt %, and sub-ranges such as 5 wt % to 15 wt %, 10 wt % to 20 wt %, etc. As used herein, “images” refers to marks, signs, symbols, figures, indications, and/or appearances deposited upon a material or substrate with either visible or an invisible ink composition. Examples of an image can include characters, words, numbers, alphanumeric symbols, punctuation, text, lines, underlines, highlights, and the like.

In some embodiments, the present disclosure provides recording media containing a raw base substrate having, on its image side, a primary coating layer and a top image-receiving layer wherein said image receiving layer encompasses a polymeric adhesion promoter having a glass transition temperature (Tg) that is at, or higher, than 90° C. In some examples, such recording or receptive media is an inkjet printable media well adapted for inkjet printing device. In some other embodiments, the present disclosure refers to a printing method for producing durable images on a recording media. Said method encompasses obtaining an inkjet recording media containing a raw base substrate having, on its image side, a primary coating layer and a top image receiving layer wherein said image receiving layer encompasses a polymeric adhesion promoter having a glass transition temperature (Tg) that is at, or above, 90° C., and jetting an ink composition containing latex onto said recording media to form a printed image with enhanced image quality and enhanced image permanence. In some examples,

the method further encompasses a drying step. In some examples, the ink composition used herein contains a latex component that is identical to the polymeric adhesion promoter present in the image receiving layer of the recording media. In yet some other embodiments, the present disclosure refers to a printed article containing the recording media such as defined herein on which a printed feature has been formed with an ink composition. Said recording media is an inkjet printable media with a raw base substrate comprising, on its image side, a primary coat layer and a top image receiving layer wherein said image receiving layer encompasses a polymeric adhesion promoter having a glass transition temperature (Tg) that is at, or above, 90° C. and wherein the ink composition encompasses latex components that have a glass transition temperature (Tg) that is at, or above, 90° C.

The recording media, the printing method and the printed article of the present disclosure have the ability to provide prints with improved printing performances, specifically improved adhesion performances to ink colorant particles. In some examples, the images printed on the recording media, such as described herein, are able to impart excellent image quality. In some other examples, the printed images impart good adhesion capability to ink colorant and latex particles when an ink composition containing latex is used for forming the printed image. The media described herein has the ability to provide excellent image quality: it has good adhesion (helps avoid ink-running issues) and has good ink water and scratch resistance. Furthermore, when used in a printing process using latex ink composition, the resulting printed image presents good wet and dry scrub strength as well as excellent ink adhesion to the surface. Indeed, without being linked by any theory, it is believed that the image durability strongly depends upon the adhesion of ink colorant and latex particles to media surface.

FIG. 1, FIG. 2 and FIG. 3 illustrate some embodiments of the recording media (100). As will be appreciated by those skilled in the art, FIG. 1, FIG. 2 and FIG. 3 illustrate the relative positioning of the various layers of the recording media (100) without necessarily illustrating the relative thicknesses of said layers. As shown in FIG. 1, FIG. 2 and FIG. 3, the recording media (100) encompasses a base substrate (110). The base substrate (110) has two surfaces: a first surface that might be referred to as the "image surface" or "image side" (101), and a second surface, the opposite surface, which might be referred to as the "back surface" or "back side" (102). Thus, the recording media (100) contains an image side (101), i.e. wherein the image is deposited, and a back side (102) which is not very well adapted to receive some image. FIG. 1 illustrates some embodiments of the recording media (100). Such media includes a primary coating layer (120) that is applied on the image side (101) of the base substrate (110). The recording media (100) further includes a top image-receiving layer (130) that is applied over the primary coating layer (120) on the image side (101) of the media. FIG. 2 illustrates some other embodiments of the recording media (100). Such media includes primary coating layers (120) that are applied on both sides of the base substrate (110). The primary coating layers (120) are thus present on the back side (102) and on the image side (101) of the base substrate (110). The recording media (100) further includes a top image-receiving layer (130) that is applied over the primary coating layer (120) on the image side (101) of the media. FIG. 3 illustrates yet some other embodiments of the recording media (100). Such recording media includes primary coating layers (120) that are applied on both sides of the base substrate (110). The primary

coating layers (120) are thus present on the back side (102) and on the image side (101) of the base substrate (110). The recording media (100) includes a top image-receiving layer (130) that is applied over the primary coating layer (120) on the image side (101) of the media and includes an adhesive layer (140) that is applied over the primary coating layer (120) on the back side (102) of the media.

FIG. 4, FIG. 5 and FIG. 6 illustrate some embodiments of the printed article (200). FIG. 4 illustrates some embodiments of the printed article (200) wherein such printed article (200) includes a recording media (100) having a primary coating layer (120), a top image-receiving layer (130) applied on the image side (101) of the base substrate (110), and includes a printed feature (210) that has been formed with an ink composition containing latex components having a glass transition temperature (Tg) that is at, or above, 90° C. FIG. 5 illustrates some other embodiments of the printed article (200), wherein such printed article (200), includes a recording media (100) having primary coating layers (120) that are applied on both sides of the base substrate (110), a top image-receiving layer (130) applied on the image side (101) of the base substrate (110), and includes a printed feature (210) that has been formed with an ink composition containing latex components having a glass transition temperature (Tg) that is at, or above, 90° C. FIG. 6 illustrates yet some other embodiments of the printed article (200), wherein such printed article (200) includes a recording media (100) having primary coating layers (120) on both sides of the base substrate (110), a top image-receiving layer (130) applied on the image side (101) over the primary coating layer (120); an adhesive layer (140) applied over the primary coating layer (120) on the back side (102) of the media and a printed feature (210) that has been formed with an ink composition containing latex components having a glass transition temperature (Tg) that is at, or above, 90° C.

In some embodiments, the recording media (100) contains a raw base substrate (110) having, on its image side, a primary coating layer (120) and a top image-receiving layer (130). In some examples, the raw base substrate (110) is a media substrate that can be a cellulose paper base, a polymeric film base or a non-organic film base. In some examples, the raw base has a base weight of about 50 to about 300 grams/meter<sup>2</sup> (gsm), and, in some other examples, the raw has a base weight of about 100 to about 220 gsm. In some embodiments, the raw base (110) is a cellulose base paper. Any kind of cellulose raw base may be used. The raw base (110) can be made of any suitable wood or non-wood pulp. Non-limitative examples of suitable pulps include any kind of chemical pulp, mechanical wood pulp, chemically treated ground pulp, CTMP (chemical thermo mechanical pulp), and/or mixtures thereof. In some examples, ground-wood pulp, sulfite pulp, chemically ground pulp, refiner ground pulp, and thermo-mechanical pulp or their mixture can thus be used. In some examples, the raw base (110) contains non-wood pulp such as pulp originating from bamboo, bagasse, kenaf, papyrus, etc. Bleached hardwood chemical pulps may make up the main pulp composition. This pulp has shorter fiber structure than soft wood, which contribute to good formation of the finished paper. Fillers may also be incorporated into the pulp, for example, to substantially control physical properties of the final coated paper. The filler particles fill in the void spaces of the fiber network and result in a denser, smoother, brighter and opaque sheet. Examples of the fillers include, but are not limited to, ground calcium carbonate, precipitated calcium carbonate, titanium dioxide, kaolin clay, silicates, plastic

## 5

pigment, alumina trihydrate, and/or mixtures thereof. It is to be understood that any desirable amount of filler, such as 15 wt %, may be used. In some examples, the amount of filler ranges from about 0.1 wt % to about 20 wt % of the raw base, and in some other examples, the amount of filler ranges from about 5 wt % to about 15 wt % of the raw base.

When preparing the paper base stock, internal sizing may be used. These processes may improve hydrophobicity of the cellulose fibers that in turn may control the resistance of the coated substrate to wetting, penetration, and absorption of aqueous liquids. Internal sizing may be accomplished by adding a sizing agent to the furnish containing fibers and fillers in the wet end. Non-limitative examples of suitable sizing agents include resin-based sizing agent(s), wax-based sizing agent(s), cellulose-reactive sizing agent(s) and other synthetic sizing agent(s), and/or mixtures. It is to be understood that the type and amount of surface sizing agent(s) may substantially improve moisture resistance. Surface sizing (i.e. apply surface sizing agents and other functional additives to the formatted paper surface) may be accomplished by any kind of sizing methods such as film size press, pond size press and other surface techniques. It is understood that any conventional size press agents, such as any kind of virgin starch, chemical, physical or biological modified starch is not suitable herein as all kind of starch species is not exactly meeting the desired water/moisture resistance. Without being bounded by any theory, it is believed that surface sizing composition plays dual roles for the substrates as both barrier function to the outside moisture and wet strength agent improve the wet strength when the substrate is subjected to high aqueous ink volume printing and afterwards water immersion, during application/installation. In some examples, a synthetic polymeric resin is used as the surface sizing agent. There are wide varieties of resin compositions that can be used for surface sizing. For example, the resin compositions may include, but are not limited to, resins formed by polymerization of hydrophobic addition monomers. Examples of hydrophobic addition monomers include, but are not limited to, C<sub>1</sub>-C<sub>12</sub> alkyl acrylate and methacrylate (e.g., methyl acrylate, ethyl acrylate, n-propyl acrylate, isopropyl acrylate, n-butyl acrylate, isobutyl acrylate, sec-butyl acrylate, tert-butyl acrylate, 2-ethylhexyl acrylate, octyl arylate, methyl methacrylate, ethyl methacrylate, n-propyl methacrylate, isopropyl methacrylate, n-butyl methacrylate, isobutyl methacrylate, sec-butyl methacrylate, tert-butyl methacrylate), and aromatic monomers (e.g., styrene, phenyl methacrylate, o-tolyl methacrylate, m-tolyl methacrylate, p-tolyl methacrylate, benzyl methacrylate), hydroxyl containing monomers (e.g., hydroxyethylacrylate, hydroxyethylmethacrylate), carboxylic containing monomers (e.g., acrylic acid, methacrylic acid), vinyl ester monomers (e.g., vinyl acetate, vinyl propionate, vinylbenzoate, vinylpivalate, vinyl-2-ethylhexanoate, vinylversatate), vinyl benzene monomer, C<sub>1</sub>-C<sub>12</sub> alkyl acrylamide and methacrylamide (e.g., t-butyl acrylamide, sec-butyl acrylamide, N,N-dimethylacrylamide), crosslinking monomers (e.g., divinyl benzene, ethyleneglycol dimethacrylate, bis(acryloylamido)methylene), and any combinations thereof. In some other examples, polymers made from the polymerization and/or copolymerization of alkyl acrylate, alkyl methacrylate, vinyl esters, and styrene derivatives may be useful. The polymers can be made using a wide variety of polymerization methods. For example, the polymers may be made using bulk polymerization, solution polymerization, emulsion polymerization, or other suitable methods. The emulsion polymerization in the presence of aqueous solvent such as water may be useful in making the

## 6

polymer resins described above. In some examples, the polymer latex resin can be made using emulsion polymerization with a particle size ranging from about 0.1 to about 5 micrometers. In some other examples, the particle size may range from about 0.5 to about 3 micrometers and, in yet some other examples, the average particles size of latex resin can be of about 1.2 micrometers.

In some embodiments, inorganic fillers can be present in surface the sizing composition. The inorganic filler in the surface sizing composition can have a mean size ranging from about 0.2 micrometers to about 1.5 micrometers. These inorganic fillers can be in a powder or slurry form, and, for examples, include, but are not limited to, titanium dioxide, hydrated alumina, calcium carbonate, barium sulfate, silica, clays (such as high brightness kaolin clays), and zinc oxide. In some examples, calcium carbonate may be used. Calcium carbonate has a number of desirable properties including high brightness, gloss, opacity, good rheology, and good coating ability. In some examples, the part number of the inorganic fillers by weight per about 100 parts of polymeric resin, is ranged from about 0 to about 10 parts, and in some other examples, from about 0.5 to no more than about 5 parts. Excessive loading of inorganic fillers will reduced the penetration capability of surface sizing composition to bulk of the base substrate wet strength of the base substrate. The z-direction penetration of the surface sizing composition might be all way to the centre of the base substrate if sizing from both side, or to reach another surface in one side sizing case. In some examples, the z-direction penetration depth is over half of  $\frac{1}{2}$  of base substrate in two sides sizing and, in some other examples, the z-direction penetration depth is over half of  $\frac{2}{3}$  of base substrate in two sides sizing. It might be not desirable that penetration depth is less than  $\frac{1}{2}$  of the half of base substrate in two sides sizing. In some examples, the thickness of the surface sizing layer ranges from about 0.01 micrometer to about 3 micrometer and, in some other examples, ranges from about 0.05 micrometer to about 1 micrometer per side of the base substrate. In order to prevent penetration of moisture into the base substrate, the surface can be sized on both sides.

In some examples, since the stiffness of the raw base may be related, at least in part, to the paper thickness, or paper weight, it is to be understood that with substantially the same pulp and filler composition, the thinner the paper caliper is, the lower the paper stiffness will be. If base weight is less than 100 gsm, low flexural rigidity may generate difficulties in paper handling during printing. Customers also have lower acceptance for such a lightweight paper as photographic printout. However, if base weight is over 300 gsm, many printers cannot support such high stiffness media. In some examples, the stiffness of the raw base ranges from about 800 Gurley stiffness units to about 2000 Gurley stiffness units in the paper machine direction, and ranges from about 300 Gurley stiffness units and about 1200 Gurley stiffness units in the paper cross machine direction. In some other examples, the base paper stiffness ranges from about 800 Gurley stiffness units to about 1500 Gurley stiffness units in the paper machine direction, and from about 350 Gurley stiffness units to about 1000 Gurley stiffness units in the paper cross machine direction. A method, such as TAPPI T543 om-94, using a Gurley-type stiffness tester, may be used to determine the stiffness of the paper stock. In some examples, when the raw base (110) is a cellulose paper base, the base substrate may have a low porosity and a strong capability to resist moisture migration in view of keeping good physical strength when the recording medium is used in an high moisture environment (such as outdoor usage). In

some examples, in view of reducing the moisture, absorption wet strength agents or internal sizing agents can be added to the raw base.

In some examples, the recording media (100) encompasses a primary coating layer (120) that is applied directly on the base stock substrates. Such as illustrated in FIG. 1, the primary coating layer (120) can be present on one side of the recording media (100), i.e. on the image side (101) of the raw base or, in some other examples, such as illustrated in FIGS. 2 and 3, the primary coating layers (120) can be present on the back side (102) and on the image side (101) of the recording media (100), i.e. on both side of the raw base (110). Without being linked by any theory, it is believed that the function of the pigmented pre-coating layer(s) (120) is to create a smooth surface to help develop superior gloss. Additionally, the pigmented pre-coating layer(s) (120) can promote improved opacity, brightness, and appropriate color hue for the print medium. Furthermore, it is believed that primary coating layers help to enhance surface energy over base stock (especially polymer saturated base stock) so that top image receiving layer can be firmly adhered to the base stock without loading any excessive additives for adhesion improvement in the image receiving coating. In some embodiments, the primary coating layer(s) (120) includes pigment fillers and binders. The primary coating layer(s) (120) can further include surfactants and can include optional other additives. In some other embodiments, the primary coating layer(s) (120) includes a mixture of calcium carbonate and clay as pigment fillers, polymer latex as binders and surfactants.

The amount of inorganic pigment particles present in the primary coating layer (120) may be from about 40 to about 95% by weight (wt %) or may be from about 60 to about 90% by weight (wt %) based on the total weight of the coating layer (120). In some examples, the amount of binders present in the primary coating layer (120) may be from about 5 to about 60% by weight (wt %) or may be from about 10 to about 40% by weight (wt %) based on the total weight of the coating layer (120). The primary coating layer(s) (120) can be applied over the raw base (110) with a coating weight of about 5 to about 30 grams/meter<sup>2</sup> (gsm), or with a coat weight ranging from about 10 to about 15 gsm. When applied to both side of the raw base (110), the coat weight of the pre-coatings layers (120) is from about 10 to about 15 gsm for each coating sides.

In some embodiments, the image side (101) of the recording media (100) encompasses an image receiving layer (130) that is applied over the primary coating layer (120). In some examples, the image receiving layer (130) has a coat weight ranging from about 1 to about 30 grams/m<sup>2</sup>; in some other examples, ranging from about 3 to about 20 grams/m<sup>2</sup> and, in yet some other examples, ranging from about 5 to about 15 grams/m<sup>2</sup>. Without being linked by any theory, it is believed that the top image receiving layer (130) is used for enhancing compatibility between the ink composition containing latex and the media surface and, consequently, to improve the adhesion between the ink composition containing latex and the printing substrate. In some embodiments, the image receiving layer (130) includes pigment filler, a binder and a polymeric adhesion promoter. In some examples, the pigment filler is inorganic pigment filler. In some other examples, the polymeric binder presents in the top image receiving layer (130) is the same as the one used in the primary layer(s) (120).

The amount of inorganic pigment particles present in the top image receiving layer (130) may be from about 50 to about 95% by weight (wt %) or may be from about 60 to

about 90% by weight (wt %) based on the total weight of the top image receiving layer (130). The amount of binders present in the top image receiving layer (130) may be from about 10 to about 30% by weight (wt %) or may be from about 15 to 25% by weight (wt %) based on the total weight of the top image receiving layer (130). The amount of polymeric adhesion promoter present in the top image receiving layer (130) may be from about 5 to 25% by weight or may be from about 10 to 20% by weight, based on the total weight of the top image receiving layer (130). In some other examples, the amount of adhesion promoter present in the top image receiving layer (130) of the recording media, is in the range of about 5 to about 30 parts, and, in some other examples, in the range of about 5 to about 15 parts per 100 parts by dry weight of inorganic filler.

In some embodiments, the top image receiving layer (130) encompasses a polymeric adhesion promoter. Without being linked by any theory, the polymeric adhesion promoter is a substance with a macro-molecular chain structure that acts at the interface of printing media surface and ink colorant/binder particles in view of increasing the adhesion of ink colorants/binders to the printing media through the reduction of the interfacial tension. There are no specific limitations on the kinds of repeat units of macro-molecular chains and/or its side function groups. The repeat units and/or the side function groups can be either reactive, non-reactive or mixture of both. In the case that they are reactive, the adhesion promoter might chemically interact with functional groups of the ink colorants and of the printing media (by forming a covalent, an ionic or both bonds). By this way, the adhesion promoter can thus reduce or eliminate the repelling effects existing between ink colorants and printing media surface. Non-reactive polymeric adhesion promoter can also improve incompatibility among ink colorants/binders and printing media surface by means of reducing interfacial energy among the components, and subsequently improving the adhesion of the printing ink on printing media.

In some embodiments, the adhesion promoter, present in the top image receiving layer (130), is a homo-polymer or a co-polymer of alkyl acrylate, alkyl methacrylate, alkyl acrylic acid, alkyl methacrylic acid, vinyl esters, and/or styrene derivatives. Such polymers can also be in a salt form 45 with either cationic or anionic charged molecules. In some examples, the adhesion promoter is selected from the group consisting of polymers based polyacrylate and/or polyacrylate copolymers. Examples include, but are not limited to, poly(methyl methacrylate-butadiene), poly(ethyl methacrylate-butadiene), poly(propyl methacrylate-butadiene), poly(butyl methacrylate-butadiene), poly(methyl acrylate-butadiene), poly(ethyl acrylate-butadiene), poly(propyl acrylate-butadiene), poly(butyl acrylate-butadiene), poly(methyl methacrylate-isoprene), poly(ethyl methacrylate-isoprene), 50 poly(propyl methacrylate-isoprene), poly(butyl methacrylate-isoprene), poly(methyl acrylate-isoprene), poly(ethyl acrylate-isoprene), poly(propyl acrylate-isoprene) and poly(butyl acrylate-isoprene), poly(styrene-butadiene), poly(methyl styrene-butadiene), poly(styrene-isoprene), poly(methylstyrene-isoprene), poly(styrene-propyl acrylate), 55 poly(styrene-butyl acrylate), poly(styrene-butadiene-acrylic acid), poly(styrene-butadiene-methacrylic acid), poly(styrene-butadiene-acrylonitrile-acrylic acid), poly(styrene-butyl acrylate-acrylic acid), poly(styrene-butyl acrylate-methacrylic acid), poly(styrene-butyl acrylate-acrylonitrile), and poly(styrene-butyl acrylate-acrylonitrile-acrylic acid).

In some examples, the polymeric adhesion promoter is a polymeric salt. The electric charge of said polymer can be neutral, cationic or anionic. In some examples, the polymer is a cationic polymer in view of having a good reaction with anionic charged ink pigments. Examples includes, but are not limited to, polymeric salts of trimethyl-ammoniumethyl acrylate, trimethyl-ammoniumethyl methacrylate, trimethyl-ammoniumethyl acrylate; trimethyl-ammonium-ethyl methacrylate, dimethyl-benzylammoniumethyl acrylate, dimethyl-benzylammoniumethyl methacrylate, dimethyl-benzylammoniumethyl methacrylate, dimethyl-butyl ammonium-ethyl acrylate, dimethyl-butylammoniumethyl methacrylate, dimethyl-hexylammoniumethyl acrylate, dimethyl-hexylammoniumethyl methacrylate, dimethyl-octylammoniumethyl acrylate, dimethyl-octyl-ammoniumethyl methacrylate, dimethyl-dodecylammoniumethyl acrylate and dimethyl-dodecylammonium ethyl methacrylate, trimethyl-(4-vinylbenzyl)ammonium, triethyl-(4-vinylbenzyl) ammonium, trimethyl-ammoniumpropyl acrylate, dimethyl-octadecyl-ammoniumethyl acrylate, and dimethyl-octadecylammoniumethyl methacrylate. The counter-ions of these cationic polymers can be chloride, bromide, methylsulfate, triflate, etc.

In some examples, the adhesion promoter is an aqueous emulsion in the form of latex particles. Such latex adhesion promoter compositions may include those prepared using emulsion co-polymerization of various ratios of monomer such as, but in no way limited to, methyl methacrylate, styrene, with various 'soft' acrylate esters, and functionalized monomers. These functionalized monomers include 'vinyl' monomers containing hydroxyl groups, carboxylic acids, sulfonic or sulfate acids and phosphate acids. As used herein, 'vinyl' denotes derivatives of acrylates, methacrylates, functionalized styrene, allyl ether and esters, vinyl ethers as selected examples. Co-polymers can be formed, including block copolymers, randomly assembled copolymers, cross-linkable copolymers, or the like. In some other examples, the adhesion promoter is a polyacrylate-styrene copolymer or a polymethyl acrylic-styrene copolymer in the form of latex particles.

Latex adhesion promoter particles can utilize a measured amount of surface acid groups to provide stability over longer periods of time (to resist aggregation) and to provide improved adhesion to certain polar interfaces. In a more detailed aspect, the latex particles can be prepared using various monomers as sources of acid functionality. In use, polymeric acid functionalities are neutralized to provide a latex particle surface charge. Acid functionality may include ionizable groups such as carboxylic acids, sulfonic or sulfate acids and phosphate acids. In some examples, the amount of the co-polymerized surface acid co-monomer can ranged from about 0.01 to about 10% of total monomers.

In some examples, the adhesion promoter is not a water soluble polymer. It is meant thus that the adhesion promoter polymer does not have a solid content change, in an aqueous solvent under room temperature and pressure that is greater than 5% by weight with a period of 24 hours. In some other examples, the adhesion promoter is a water dispersible polymer. The adhesion promoter can be dispersed into small particles of diameter in the range of about 100 to about 500 nanometer (nm), with or without external shear force, in view of forming a stable emulsion with or without aid of an emulsifier. Alternatively, in some examples, the adhesion promoter can form in-situ latex particles via emulsion polymerization with particle size in the range of about 100 to about 500 nanometer (nm). In some examples, the adhesion promoter is an acrylic latex composition in the form of latex particles. In some examples, the adhesion promoter can

have a molecular weight in the range of about 10,000 Mw to about 5,000,000 Mw as measured by GPC. In some example, the adhesion promoter polymer has a glass transition temperature (Tg) that is at 90° C., or higher than 90° C. In some other examples, the adhesion promoter polymer has a glass transition temperature (Tg) that is at 95° C., or higher, than 95° C. The way of measuring the glass transition temperature (Tg) parameter is described in, for example, Polymer Handbook, 3rd Edition, authored by J. Brandrup, 10 edited by E. H. Immergut, Wiley-Interscience, 1989.

Latexes include both latex particulates as well as the aqueous medium in which the latex particulates are dispersed. More specifically, latex is a liquid suspension comprising a liquid (such as water and/or other liquids) and polymeric particulates ranging from about 20 nm to about 15 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040 10045 10050 10055 10060 10065 10070 10075 10080 10085 10090 10095 10100 10105 10110 10115 101

## 11

decreased to the level which normal coating binder has, it will adversely soften latex ink film and make printing durability decreasing.

In some examples, the primary coating layer(s) (120) and the top image receiving layer (130) include, at least, one filler. The filler, used in the top image receiving layer (130), is independently selected from the one used in the primary coating layer(s) (120). The primary coating layer(s) (120) and the top image receiving layer (130) can include a mixture of two or more pigment fillers with different particle size and size distribution. In some examples, such fillers are inorganic pigments. Examples of inorganic pigments include metal oxides and/or semi-metal oxides particles. The inorganic pigments may also be independently selected from the group consisting of calcium carbonate, zeolite, silica, talc, alumina, boehmite, silicates (such as aluminum silicate, magnesium silicate and the like), aluminum trihydrate (ATH), titania, zirconia, clays, calcium silicate, kaolin, calcined clay or combinations thereof. In some examples, the inorganic pigments are calcium carbonate, precipitated calcium carbonate, ground calcium carbonate, kaolin clays, and others. The physical form of the pigments can be either powder or aqueous pre-dispersed slurry. Optionally, co-pigments can be present in the primary coating layer(s) (120) and in the top image receiving layer (130). Such co-pigments include, for example, pigments that have both a micro-porous structure, such as fumed silica and silica gels, and "structured" pigments. Examples of these structured pigments are calcined clays and porous clays/calcium carbonate that are reaction products of clay/calcium carbonate with colloidal silica. Other inorganic particles such as particles of titanium dioxide ( $TiO_2$ ), silicon dioxide ( $SiO_2$ ), aluminum trihydroxide (ATH), calcium carbonate ( $CaCO_3$ ) and zirconium oxide ( $ZrO_2$ ) can be inter-calcined into the structured clay or calcium carbonates. Co-pigment particles may be substantially non-porous mineral particles that have a special morphology that can produce a porous coating structure when solidified into a coating layer. In some examples, such particles are aragonite precipitated calcium carbonates. In some other examples, the particles have a needle-like structure on a microscopic scale, i.e. they have a high aspect (length-to-width) ratio. This structure results in a loose coating layer packing with a relatively large fraction of voids on the coating surface.

In some examples, the primary coating layer(s) (120) and the top image receiving layer (130) include, at least, a polymeric binder. The polymeric binder of the top image receiving layer (130) is independently selected from the one used in the primary coating layer(s) (120). In some examples, the polymeric binder can be either water a soluble, a synthetic or a natural substances or an aqueous dispersible substance like polymeric latex. In some other examples, the polymeric binder is polymeric latex. Without being linked by any theory, it is believed that the polymeric binder is used to provide adhesion among the inorganic particles and other components within the image receiving layer (130) and within the primary coating layer(s) (120). The polymeric binder is also used to provide adhesion between the image receiving layer (130) and the primary coating layer(s) (120), as well as the adhesion between primary coating layer(s) and base substrate (110). The polymeric binder can be a water soluble polymer or water dispersible polymeric latex. In some examples, the binder is selected from natural macromolecule materials such as starches, chemical or biological modified starches and gelatins. The binder may be selected from the group consisting of water-soluble binders and water dispersible polymers that

## 12

exhibit high binding power for base paper stock and pigments, either alone or as a combination. In some examples, the polymeric binder components have a glass transition temperature (Tg) ranging from  $-10^\circ C$ . to  $+50^\circ C$ . The way of measuring the glass transition temperature (Tg) parameter is described in, for example, Polymer Handbook, 3rd Edition, authored by J. Brandrup, edited by E. H. Immergut, Wiley-Interscience, 1989.

Suitable binders include, but are not limited to, water soluble polymers such as polyvinyl alcohol, starch derivatives, gelatin, cellulose derivatives, acrylamide polymers, and water dispersible polymers such as acrylic polymers or copolymers, vinyl acetate latex, polyesters, vinylidene chloride latex, styrene-butadiene or acrylonitrile-butadiene copolymers. Non-limitative examples of suitable binders include styrene butadiene copolymer, polyacrylates, polyvinylacetates, polyacrylic acids, polyesters, polyvinyl alcohol, polystyrene, polymethacrylates, polyacrylic esters, polymethacrylic esters, polyurethanes, copolymers thereof, and combinations thereof. In some examples, the binder is a polymer and copolymer selected from the group consisting of acrylic polymers or copolymers, vinyl acetate polymers or copolymers, polyester polymers or copolymers, vinylidene chloride polymers or copolymers, butadiene polymers or copolymers, styrene-butadiene polymers or copolymers. In some other examples, the binder component is a latex containing particles of a vinyl acetate-based polymer, an acrylic polymer, a styrene polymer, an SBR-based polymer, a polyester-based polymer, a vinyl chloride-based polymer, or the like. In yet some other examples, the binder is a polymer or a copolymer selected from the group consisting of acrylic polymers, vinyl-acrylic copolymers and acrylic-polyurethane copolymers. Such binders can be polyvinylalcohol or copolymer of vinylpyrrolidone. The copolymer of vinylpyrrolidone can include various other copolymerized monomers, such as methyl acrylates, methyl methacrylate, ethyl acrylate, hydroxyethyl acrylate, hydroxyethyl methacrylate, ethylene, vinylacetates, vinylimidazole, vinylpyridine, vinylcaprolactams, methyl vinylether, maleic anhydride, vinylamides, vinylchloride, vinylidene chloride, dimethylaminoethyl methacrylate, acrylamide, methacrylamide, acrylonitrile, styrene, acrylic acid, sodium vinylsulfonate, vinylpropionate, and methyl vinylketone, etc. Examples of binders include, but are not limited to, polyvinyl alcohols and water-soluble copolymers thereof, e.g., copolymers of polyvinyl alcohol and poly(ethylene oxide) or copolymers of polyvinyl alcohol and polyvinylamine; cationic polyvinyl alcohols; aceto-acetylated polyvinyl alcohols; polyvinyl acetates; polyvinyl pyrrolidones including copolymers of polyvinyl pyrrolidone and polyvinyl acetate; gelatin; silyl-modified polyvinyl alcohol; styrene-butadiene copolymer; acrylic polymer latexes; ethylene-vinyl acetate copolymers; polyurethane resin; polyester resin; and combination thereof. Examples of binders include Poval® 235, Mowiol® 56-88, Mowiol® 40-88 (products of Kuraray and Clariant).

The binder may have an average molecular weight (Mw) of about 5,000 to about 500,000. In some examples, the binder has an average molecular weight (Mw) ranging from about 100,000 to about 300,000. In some other examples, the binder has an average molecular weight of about 250,000. The average particle diameter of the latex binder can be from about 10 nm to about 10  $\mu m$ ; in some other examples, from about 100 nm to about 5  $\mu m$ ; and, in yet other examples, from about 500 nm to about 0.5  $\mu m$ . The particle size distribution of the binder is not particularly limited, and

either binder having a broad particle size distribution or binder having a mono-dispersed particle size distribution may be used. The binder may include, but is in no way limited to latex resins sold under the name Hycar® or Vycar® (from Lubrizol Advanced Materials Inc.); Rhoplex® (from Rohm & Hass company); Neocar® (from Dow Chemical Comp); Aquacer® (from BYC Inc) or Lucidene® (from Rohm & Haas company).

The primary coating layer(s) (120) and the top image receiving layer (130) may further include optional additives such as mordants, biocides, surfactants, plasticizers, rheology modifiers, defoamers, optical brighteners, pH controlling agents, and other additives for further enhancing the properties of the coating. Among these additives, rheology modifier is useful for addressing runnability issues. Suitable rheology modifiers include polycarboxylate-based compounds, polycarboxylated-based alkaline swellable emulsions, or their derivatives. The rheology modifier is helpful for building up the viscosity at certain pH, either at low shear or under high shear, or both. In certain embodiments, a rheology modifier is added to maintain a relatively low viscosity under low shear, and to help build up the viscosity under high shear. It is desirable to provide a coating formulation that is not so viscous during the mixing, pumping and storage stages, but possesses an appropriate viscosity under high shear. Some examples of rheology modifiers that meet this requirement include, but are not limited to, Sterocoll® FS (from BASF), Cartocoat® RM 12 (from Clariant), Acrysol® TT-615 (from Rohm and Haas) and Acumer® 9300 (from Rohm and Haas). The amount of rheology modifier in the coating composition may be in the range of about 0.1 to about 2 parts, in some other examples, in the range of about 0.1 to about 0.5 parts based on 100 parts of inorganic pigments. In some embodiments, the primary coating layer(s) (120) includes surfactants. There is no specific limitation on the chemical structure of surfactant used in the primary coating layer. In some examples, poly-alkylene oxide based surfactant such as Surfynol® (supplied by Air Product), or the silicone base surfactants (BYK® surfactants supplied by BYK Inc) can be used in said coating layer.

In some examples, the recording media (100) encompasses on the back side (102) of the raw base substrate (110), an adhesive layer (140). Such as illustrated in FIG. 3, the adhesive layer (140) can be present on the back side (102) of the raw base substrate (110) above the primary coating layer (120). Such adhesive coating layer (140) can contain partially water soluble macromolecules chemicals such as partially esterified polyvinyl alcohol, partially cross-linked PVA with low or medium molecular weight, and chemical modified starches. In some examples, polyacrylic acid and cross-linked polyacrylic acid can be present in the adhesive layer (140). In some other examples, inorganic filler can be present in an amount representing less than about 50% by weight of the total adhesive layer. Some functional additives, such as surface color dye and PH adjuster, can also be present. Without being linked by any theory, it is believed that the function of the adhesive coating layer (140) is to create some conveniences to the end user of the printing products who can, for example, readily place the printed media on any substrate like wall, glass surface, paper or plastic broad for displaying. In some examples, such adhesive layer helps the printed media to be "removable or repositionable" (like a sticker). In some other examples, such adhesive layer make the printed media "strippable", meaning thus that the printed media can be easily removed

from any substrate (like a wall) without damage the substrate located below, such as the painting.

In some embodiments, the present disclosure refers to a method of making a recording media. Such method encompasses applying a primary coating layer (120) on the image side of a raw base substrate (110); drying the primary coating layer (120); applying a top image receiving layer (130) over said primary coating layer, drying and calendering said layers. In some other examples, the method encompasses: applying primary coating layers (120) on both side of a raw base substrate (110); drying the primary coating layers (120); applying a top image receiving layer (130) over one side of said a primary coating layer, drying and calendering said layers. In both methods, the image receiving layer (130) encompasses polymeric adhesion promoter with a glass transition temperature (Tg) that is at 90° C. or higher than 90° C. In yet some other examples, an adhesive layer (140) is applied on the back side (102) of a raw base substrate (110), over the primary coating layer (120).

The primary coating layer(s) (120), the top image receiving layer (130) and adhesive layer (140), when present, may be applied to the supporting substrate (110) using any one of a variety of suitable coating methods, such as blade coating, air knife coating, metering rod coating, curtain coating, or another suitable technique. In some examples, blade-coating, metering rod coating or run the coating process at high speed are used. For a double-side coated medium, depending on the set-up of production machine in a mill, both sides of the substrate may be coated during a single manufacture pass, or alternatively, each side may be coated in separate passes. After the coating step, the coated medium can be subjected to a drying process to remove water and other volatile components in the coating layers and substrate. The drying means includes, but are not limited to, infrared (IR) dryers, hot surface rolls, and hot air floatation dryers. After coating, the coated medium may be calendered to increase glossiness and/or to impart a satin surface. When a calendering step is incorporated, the coated medium may be calendered by an on-line or an off-line calender machine, which may be a soft-nip calender or a super-calender. The rolls, in a calendar machine, may or may not be heated, and pressure is usually applied to the calendering rolls. In some examples, the primary coating layer(s) (120), the top image receiving layer (130) and the adhesive layer (140) are coated onto the base substrate (110) using any method known in the art including size press, slot die, curtain coating, blade coating and Meyer rod. The size presses include puddle-sized press, film-sized press and the like. The puddle-sized press can be configured as having horizontal, vertical, or inclined rollers. The film-sized press can include a metering system, such as gate-roll metering, blade metering, Meyer rod metering, or slot metering. In some examples, a film-sized press with short-dwell blade metering can be used as an application head to apply a coating solution. In some examples, a film-sized press is used to apply the ink receiving layer (130) to a paper substrate. The image receiving layer (130) can be applied to paper substrate off-line or in-line of a paper-making machine.

In some embodiments, the present disclosure refers to a printing method for producing durable images on a recording media such as defined above. In some examples, said method encompasses: obtaining a recording media containing a raw base substrate (110) having, on its image side, a primary coating layer (120) and a top image receiving layer (130) wherein said image receiving layer encompasses a polymeric adhesion promoter having a glass transition temperature (Tg) ranging at, or above, 90° C.; jetting an ink

composition containing latex onto said recording media, to form a printed image with enhanced image quality and enhanced image permanence. Said method might further encompass the step of drying the printed image. In some examples, the polymeric adhesion promoter is in the form of latex particles having a size ranging from about 150 to about 350 nanometers with a glass transition temperature ranging at, or above, 90 degrees C. In some other embodiments, the ink composition used in said method, contains a latex component that is identical to the polymeric adhesion promoter present in the image receiving layer (130).

The recording media according to embodiments of the present disclosure, when used in inkjet printing with ink composition containing latex, imparts good image quality, improved durability and excellent adhesion performances. Without being bound by the theory, it is believed that the polymer adhesion promoter present in the recording media, when used in printing method using latex-based inks (i.e. printed with ink composition containing latex), act synergistically with the ink composition containing latex in view of providing printed image with improved adhesion property. The printed image will have a superior adherence and enhanced image permanence when printed in such recording media. Furthermore, when the ink composition encompasses a latex component that is identical to the polymeric adhesion promoter present in the top image receiving layer (130), the resulting printed image provides enhanced inkjet image quality and enhanced image permanence.

The polymers adhesion promoter present in the image receiving layer (130) of the recording media, provides thus media having the good capacity for receiving and retaining the ink. When printed with ink compositions containing latex, embodiments of the inkjet recording media provides good image quality and enhanced image adhesion to said media. Thus, the recording media (100), when used in an inkjet printing process, provides good image quality and has a structure which is receptive and which presents excellent adherence properties to the ink deposited thereon. In some examples, the present disclosure relates thus to a method for forming printed images on ink recording media such as defined herein, using a inkjet ink composition containing latex. In some other examples, the method of forming printed images on ink recording media, such as defined herein, using the latex ink composition is done in a heated environment. The method encompasses the step of projecting a stream of droplets of the ink composition onto said ink recording media to form the desired printed image. The ink composition containing latex may be established on the media via any suitable inkjet printing technique. Non-limitative examples of such inkjet printing techniques include thermal, acoustic, continuous and piezoelectric inkjet printing. In some embodiments, the inkjet recording media is used with any suitable inkjet printer and with any ink composition containing latex that is ordinarily used for inkjet printing. Examples of such printers are HP L25500 and HP L65500 (Hewlett-Packard Corporation).

By inkjet composition, it is meant herein that the composition is very well adapted to be used in an inkjet printing device and/or in an inkjet printing process. As latex ink composition or latex-based ink composition, it is meant herein an ink composition containing polymeric latex. Thus, in some embodiments, the media of the present disclosure is used in combination with an ink composition containing latex. The ink composition used herein is, therefore, a composition comprising polymeric latex. In some examples, the polymeric latex is suspended or dissolved in an ink vehicle. In some examples, the inkjet ink composition

containing latex encompasses polymeric latex. The polymeric latex refers herein to a group of preparations consisting of stable dispersion of polymeric micro-particles dispersed in the aqueous vehicle of the ink. The polymeric latex can be natural latex or synthetic latex. Synthetic latexes are, usually, produced by emulsion polymerization using a variety of initiators, surfactants and monomers. In some examples, the polymeric latex is cationic, anionic, or amphoteric polymeric latex. Any latex polymer commercially available can be used in the inks described herein including self-dispersed and functionalized latex polymers. Latex polymers can be prepared using any of a number of known emulsion polymerization techniques where co-monomers are dispersed and polymerized in a discontinuous phase of an emulsion. Monomers that are often used include ethyl acrylate; ethyl methacrylate; benzyl acrylate; benzyl methacrylate; propyl acrylate; propyl methacrylate; iso-propyl acrylate; iso-propyl methacrylate; butyl acrylate; butyl methacrylate; hexyl acrylate; hexyl methacrylate; octadecyl methacrylate; octadecyl acrylate; lauryl methacrylate; lauryl acrylate; hydroxyethyl acrylate; hydroxyethyl methacrylate; hydroxyhexyl acrylate; hydroxyhexyl methacrylate; hydroxyoctadecyl acrylate; hydroxyoctadecyl methacrylate; hydroxylauryl methacrylate; hydroxylauryl acrylate; phenethyl acrylate; phenethyl methacrylate; 6-phenylhexyl acrylate; 6-phenylhexyl methacrylate; phenyllauryl acrylate; phenyllauryl methacrylate; 3-nitrophenyl-6-hexyl methacrylate; 3-nitrophenyl-18-octadecyl acrylate; ethyleneglycol dicyclopentyl ether acrylate; vinyl ethyl ketone; vinyl propyl ketone; vinyl hexyl ketone; vinyl octyl ketone; vinyl butyl ketone; cyclohexyl acrylate; methoxysilane; acryloxypropylmethyldimethoxysilane; trifluoromethyl styrene; trifluoromethyl acrylate; trifluoromethyl methacrylate; tetrafluoropropyl acrylate; tetrafluoropropyl methacrylate; heptafluorobutyl methacrylate; iso-butyl acrylate; iso-butyl methacrylate; 2-ethylhexyl acrylate; 2-ethylhexyl methacrylate; iso-octyl acrylate; and iso-octyl methacrylate.

In some examples, the latexes used herein are prepared by latex emulsion polymerization, and, in some other examples, have a weight average molecular weight ranging from about 10,000 Mw to about 5,000,000 Mw. In some examples, the polymeric latex is selected from the group consisting of acrylic polymers or copolymers, vinyl acetate polymers or copolymers, polyester polymers or copolymers, vinylidene chloride polymers or copolymers, butadiene polymers or copolymers, styrene-butadiene polymers or copolymers, acrylonitrile-butadiene polymers or copolymers. In some examples, the polymeric latex liquid suspension contains a liquid (such as water and/or other liquids) and polymeric latex particulates having a size ranging from about 20 nm to about 500 nm. In some other examples, the polymeric latex particulates have a size ranging from about 100 nm to about 300 nm. In yet some other examples, the polymeric latex particulates have a weight average molecular weight ranging from about 10,000 Mw to about 5,000,000 Mw, or, ranging from about 40,000 Mw to about 100,000 Mw.

The ink composition can contain polymeric latex particulates in an amount representing from about 0.5 wt % to about 15 wt % based on the total weight of the ink composition. The polymeric latex particulates might contain a plurality of monomers that are often randomly polymerized, and that can be crosslinked. When crosslinked, the molecular weight can be even higher than the molecular weight cited above. Examples of polymeric latex particulates that can be used include those prepared using a mix of monomer of various weight ratios. Examples of such monomers include styrene, hexyl methacrylate, ethylene glycol dimethacrylate and

methacrylic acid. All these monomers could be copolymerized to form latex. In some examples, polymeric latex particulates contain styrene and hexyl methacrylate monomers that can provide the bulk of the latex particulate, and ethylene glycol dimethacrylate and methyl methacrylate that can be copolymerized therewith in smaller amounts. In such examples, the acid group is provided by the methacrylic acid. Other combinations of monomers can similarly be used to form latex particulates. Non-limiting examples of monomers that can be used to form such particulates include, but are in no way limited to, styrenes,  $C_1$  to  $C_8$  alkyl methacrylates,  $C_1$  to  $C_8$  alkyl acrylates, ethylene glycol methacrylates and dimethacrylates, methacrylic acids, acrylic acids, and the like.

In some embodiments, the ink composition includes polymeric latex that have a particle size ranging from about 150 to about 350 nanometers and that have a glass transition temperature ( $T_g$ ) ranging at or above 90 degrees C. In some other examples, the latex component of the ink composition is identical to the polymeric adhesion promoter component that is present in the top image receiving layer (130) of the recording media on which the ink is printed onto. In some other examples, the latex component of the ink composition is a polyacrylate-styrene copolymer or a polymethyl acrylic-styrene copolymer. In some examples, the difference of solubility parameters between ink latex binder and polymeric adhesion promoter is less than  $0.8 \text{ (cal}\cdot\text{cm}^{-3}\text{)}^{1/2}$ , and, in some other examples, is less than  $0.2$  to  $0.5 \text{ (cal}\cdot\text{cm}^{-3}\text{)}^{1/2}$ . The test is based on "Estimation of polymer solubility parameters by Inverse gas chromatography", *Macromolecular* 1982, 15, 622-624.

Without being linked by any theory, it is believed that, when the ink composition containing latex is jetted onto the recording media such as defined herein, discrete polymer particles are laid down on the media surface followed up by a drying processing. It is also believed that, when aqueous solvent is lost from the drops while ink drying, the mutual repulsive forces, associated with the surfactants, inhibit the close packing of the particles and a cubic arrangement of the particles is firstly formed. As the aqueous solvent continues to evaporate, the particles become close packed with a solids volume of around 70% or higher. When most of the water is lost from the system, the inter-particular repulsive forces are overcome by increasing surface tension and the particles coalesce into a discrete film. The film-forming depends then upon the elastic modulus of the ink latex as the resistance to particle deformation.

In some examples, the ink composition referred herein contains one or more colorants that impart the desired color to the printed message. As used herein, "colorant" includes dyes, pigments, and/or other particulates that may be suspended or dissolved in an ink vehicle. The colorant can be present in the ink composition in an amount required to produce the desired contrast and readability. In some other examples, the ink compositions include pigments as colorants. Pigments that can be used include self-dispersed pigments and non self-dispersed pigments. Any pigment can be used; suitable pigments include black pigments, white pigments, cyan pigments, magenta pigments, yellow pigments, or the like. Pigments can be organic or inorganic particles as well known in the art. As used herein, "liquid vehicle" is defined to include any liquid composition that is used to carry colorants, including pigments, to a substrate. A wide variety of liquid vehicle components may be used and include, as examples, water or any kind of solvents. Such liquid vehicles may further include a mixture of different agents, including without limitation, surfactants, solvents

and co-solvents, buffers, biocides, viscosity modifiers, sequestering agents, stabilizing agents and water. Though not liquid per se, the liquid vehicle can also carry other solids, such as polymers, UV curable materials, plasticizers, salts, etc.

In some embodiments, such as illustrated in FIGS. 4, 5 and 6, the present disclosure refers to a printed article (200) containing a recording media (100), such as defined herein, on which a printed feature (210) has been formed with an ink composition containing latex. Said recording media is an inkjet recording media with a raw base substrate (110) comprising, on its image side, a primary coat layer (120) and a top image receiving layer (130) wherein said image receiving layer encompasses a polymeric adhesion promoter having a  $T_g$  that is at, or above, 90° C. The ink composition, used to print the printed feature (210), encompasses latex components that have a glass transition temperature ( $T_g$ ) that is at, or above, 90° C. In some examples, the printed feature (210) is printed over the printed media (100), such as defined herein, and has been formed with an ink composition containing a latex component wherein the difference of solubility parameters between the latex component of the ink composition and the polymeric adhesion promoter, of the inkjet recording media, is less than  $0.8 \text{ (cal}\cdot\text{cm}^{-3}\text{)}^{1/2}$ . In some other examples, printed feature (210) is printed over the printed media (100) such as defined herein and has been formed with an ink composition containing a latex component, wherein said latex component is identical to the polymeric adhesion promoter present in the image receiving layer of the inkjet recording media.

## EXAMPLES

### Ingredients:

Pluronic® L61 is a surfactant available from BASF  
 Dynwet® 800 is a surfactant available from BYK Inc.  
 BYK® 024 is a defoamer available from BYK Inc.  
 Ammonium Hydroxide is a pH adjuster.  
 Acrumer® 9300 is a dispersing agent available from Dow Co.  
 Hydrocarb® H60 is coarse  $\text{CaCO}_3$  slurry available from Omya Inc.  
 Hydrocarb® H90 is Fine  $\text{CaCO}_3$  slurry available from Omya Inc.  
 Joncryl® 98 is Polyacrylate copolymer latex available from BASF Co.  
 All Purpose Cleaner® is a mixture containing dimethyl benzyl ammonium chloride and alkyl compounds available from Clorox Co  
 Crodafos® N-3 acid is available from Croda Inc.  
 Tergitol® 15s12 is a surfactant available from Talas Inc.  
 Chemguard S550® is a fluorosurfactant available from Chemguard.  
 MPDiol Glycol is 2-methyl-1,3-propanediol available from Lyondell Basell.  
 Cab-O-Jet® 300 is a self dispersed pigment available from Cabot Corporation

### Example 1—Preparation of Recording Media

Recording media, according to the present disclosure, and comparative media are prepared. Media A, B and C are ink recording media such as described in the present disclosure. Media D, E and F are comparative media. Media A to F are prepared, each including a base paper substrate, a primary coating layer and a top image receiving layer.

The base paper stocks used in the recording media A, B, C, D, E and F are made from cellulose fibers which contains about 78 wt % virgin fibers, about 10 wt % of post-consume fibers and about 12 wt % of calcium carbonate fillers. The base paper stock is then surface sized using an acrylic latex resin. The basis weight of the base paper stock is 165 gsm. The media is then coated, on both sides, with a primary coating layer using a pilot coater equipped with a rod measuring device. The primary coating layer contains about 85 parts by weight of calcium carbonate fillers, about 15 parts by weight of polymeric latex binder with acrylic-styrene copolymer and about 5 parts by weight of additives. (The additives include Pluronic® L61, Dynwet® 800, BYK® 024, Ammonium Hydroxide, Propylene Glycol and Acrumer® 9300). A top image receiving layer is then applied, using a pilot coater equipped with rod measuring device, running at a speed of 800 ft/min, on the image side of the media. Different image-receiving layer compositions are prepared in accordance with the formula such as illustrated in the TABLE 1 below. All amounts are expressed in parts by weight. The image receiving layers are then coated on the recording media in view of producing recording media A, B, C, D, E and F. Different Polymeric adhesion promoters (I, II, III and IV) are used.

TABLE 1

| Image receiving layer formulation | A   | B   | C   | D   | E   | F   |
|-----------------------------------|-----|-----|-----|-----|-----|-----|
| Hydrocarb ®H60                    | 90  | 90  | 90  | 90  | 90  | 90  |
| Hydrocarb ®H90                    | 10  | 10  | 10  | 10  | 10  | 10  |
| Joncryl ®98                       | 18  | 18  | 18  | 18  | 18  | 18  |
| Polymeric adhesion promoter I     | 10  | —   | 15  | —   | —   | —   |
| Polymeric adhesion promoter II    | —   | 10  | —   | —   | —   | —   |
| Polymeric adhesion promoter III   | —   | —   | —   | —   | 10  | —   |
| Polymeric adhesion promoter IV    | —   | —   | —   | —   | —   | 10  |
| Dynwet ®800                       | 0.5 | 0.5 | 0.5 | 0.5 | 0.5 | 0.5 |
| BYK ®024                          | 0.1 | 0.1 | 0.1 | 0.1 | 0.1 | 0.1 |

TABLE 2 illustrates some parameters in relation with the polymeric adhesion promoters I, II, III and IV: chemical structure, Tg and Delta (in relation with solubility parameters). The Delta (solubility parameter) represents the difference of solubility parameters between the latex part of the ink composition (used to be printed onto the media) and the polymeric adhesion promoter present in the recording media. This means thus that, when the polymeric adhesion promoter is identical to the latex in ink formulation, the value of the Delta solubility parameters is 0 (as illustrates with the polymeric adhesion promoter I). The Delta is expressed in  $(\text{cal}\cdot\text{cm}^{-3})^{1/2}$ . The solubility parameters test is based on "Estimation of polymer solubility parameters by Inverse gas chromatography", Macromolecular 1982, 15, 622-624.

TABLE 2

| Polymeric adhesion promoter | Chemical definition                                | Tg (° C.) | Delta (solubility parameter) |
|-----------------------------|----------------------------------------------------|-----------|------------------------------|
| I                           | Polyacrylate-styrene copolymer in latex form.      | +90° C.   | 0                            |
| II                          | Polymethyl acrylic-styrene copolymer in latex form | +92° C.   | 0.3                          |

TABLE 2-continued

| Polymeric adhesion promoter | Chemical definition                          | Tg (° C.) | Delta (solubility parameter) |
|-----------------------------|----------------------------------------------|-----------|------------------------------|
| III                         | Polybutyl-styrene copolymer in latex form    | -5° C.    | 0.2                          |
| IV                          | Water dispersed polymer with epoxy structure | +90° C.   | 1.8                          |

## Example 2—Recording Media Performances

Recording media A to F, obtained in Example 1, are evaluated for their printing performances, specifically for their ink adhesion performances. Media A to F are tested in combination with the black ink such as illustrated in TABLE 3 below. All percentages are expressed in percentage by weight (wt %) based on the total weight of the ink composition. The latex component of the ink composition is a polyacrylate-styrene copolymer in latex form (i.e. the polymeric adhesion promoter of formula I).

TABLE 3

| Component           | Amount (wt %) |
|---------------------|---------------|
| Cab-O-Jet ® 300     | 3.50          |
| Latex component     | 8.00          |
| 2-Pyrrolidone       | 16.00         |
| MPDiol              | 9.00          |
| Chemguard S-550 ®   | 0.75          |
| Crodafos ® N-3 acid | 0.20          |
| Tergitol ® 15s12    | 0.35          |
| Water               | Up to 100     |

An identical image sequence is printed on the recording media A, B, C, D, E and F with the black ink of TABLE 3, using a HP DesignJet L25500 Printer, (equipped with HP 789 ink cartridges). The printer is set with a heating zone temperature at about 50° C., a cure zone temperature at about 110° C., and an air flow at about 15%. Adhesion tests and ink running test are performed onto the printed media.

The ink adhesion tests are done using an abrasion scrub tester (per ASTM D4828 method). Both print sample and test probe are immerse in water or in an organic solvent (409 All Purpose Cleaner®). The amount of the ink remaining on the printed media is determined by measurement of the ink OD transferred on test probe. Good adhesion, upon immersion, will tend not to transfer ink from a printed image and the black optical density (KOD) will be maintained (A high OD indicates a worse ink adhesion). The ink water durability (or ink running test) is determined by immersing the printed sample into water and soaking it for 2 min. The ink running results are then visually evaluated after scratching the printing surface with a wet sponge followed by a shear force scratching using a striper. For ink running performances, each sample is ranked against other samples, and is then labeled with a relative score wherein: 5 is given to sample having no visible ink running; 4 to sample having very minor ink running; 3 to sample having minor ink running with acceptable level; 2 to sample having ink running at reject level; and 1 to sample having significant ink running.

Image quality is determined in terms of parameters such as gamut, black and color ink density, L\*min, ink bleed level and ink coalescence. The image gamut, black and color ink density, L\*min and black optical density (KOD) are measured on Macbeth® TD904 (Macbeth Process measure-

ment). The image quality of the prints related with ink migration such as bleeding and coalescence, are evaluated visually from the printed samples.

The results are illustrated in TABLE 4. According to these results, it is clear that good printing performances are obtained when the recording media contains polymeric ink adhesion promoter such as described herein.

TABLE 4

|         | Ink running | Ink adhesion (ink OD) in water | Ink adhesion (ink OD) in 409 cleaner ® | Coalescence | Gamut  |
|---------|-------------|--------------------------------|----------------------------------------|-------------|--------|
| A       | 5           | 3.0                            | 4.2                                    | Good        | 347500 |
| B       | 5           | 3.6                            | 4.0                                    | Good        | 346000 |
| C       | 4+          | 4.1                            | 4.2                                    | good        | 347100 |
| Comp. D | 4           | 3.7                            | 13.2                                   | good        | 345200 |
| Comp. E | 5           | 4.6                            | 9.8                                    | good        | 345800 |
| Comp. F | 3           | 5.9                            | 15.2                                   | good        | 348800 |

The invention claimed is:

1. A recording media, comprising:

a raw base substrate having an image side;  
a primary coating layer disposed on the image side, wherein the primary coating layer has a coating weight of from about 10 gsm to about 30 gsm, and the primary coating layer comprises:  
inorganic pigment particles in an amount of from about 60 wt % to about 90 wt % based on a total weight of the primary coating layer; and

a binder in an amount of from about 10 wt % to about 40 wt % based on the total weight of the primary coating layer;

a top image receiving layer disposed on the primary coating layer, the image receiving layer comprising a polymeric adhesion promoter formed from an aqueous emulsion having a minimum film forming temperature (MFPT) at, or not less, than 80° C., and including latex particles having a particle size from about 150 to about 350 nanometers, the latex particles having a glass transition temperature at, or above, 90° C.; and  
an ink composition disposed on the top image receiving layer, the ink composition comprising a latex component.

2. The recording media of claim 1 wherein the image receiving layer further comprises:

a pigment consisting of an inorganic pigment filler present in an amount of from about 60 wt % to about 80 wt % of a total weight of the image receiving layer; and  
a polymeric binder having a glass transition temperature of from -10° C. to 50° C., and present in an amount of from about 10 wt % to about 30 wt % of the total weight of the image receiving layer;  
wherein the polymeric adhesion promoter is present in an amount of about 5 parts to about 30 parts per 100 parts by dry weight of the inorganic pigment filler, the polymeric adhesion promoter having a molecular weight in the range of about 10,000 Mw to about 5,000,000 Mw as measured by GPC.

3. The recording media of claim 2 wherein:  
the inorganic pigment filler is selected from the group consisting of calcium carbonate, zeolite, silica, talc, alumina, boehmite, silicates, aluminum trihydrate, titania, zirconia, calcium silicate, kaolin, calcined clay, and combinations thereof; and  
the polymeric binder is selected from the group consisting of a styrene butadiene copolymer, polyacrylates, poly-

vinylacetates, polyacrylic acids, polyesters, polyvinyl alcohol, polystyrene, polymethacrylates, polyacrylic esters, polymethacrylic esters, polyurethanes, copolymers thereof, and combinations thereof.

4. A recording media, comprising:

a raw base substrate having an image side;  
a primary coating layer disposed on the image side;  
a top image receiving layer disposed on the primary coating layer, the image receiving layer comprising:  
a polymeric adhesion promoter formed from an aqueous emulsion having a minimum film forming temperature (MFPT) at, or not less, than 80° C., and including latex particles having a glass transition temperature at, or above, 90° C., the polymeric adhesion promoter having a molecular weight in a range of about 10,000 Mw to about 5,000,000 Mw as measured by GPC;

a pigment consisting of an inorganic pigment filler present in an amount of from about 60 wt % to about 80 wt % of a total weight of the image receiving layer; and  
a polymeric binder having a glass transition temperature of from -10° C. to 50° C., and present in an amount of from about 10 wt % to about 30 wt % of the total weight of the image receiving layer;

wherein the polymeric adhesion promoter is present in an amount of about 5 parts to about 30 parts per 100 parts by dry weight of the inorganic pigment filler; and

an ink composition disposed on the top image receiving layer, the ink composition comprising a latex component;

wherein the polymeric adhesion promoter has no binding power to the inorganic pigment filler, to the primary coating layer and to the raw base substrate at room temperature;

and wherein the polymeric adhesion promoter is selected from the group consisting of poly(methyl methacrylate-butadiene), poly(ethyl methacrylate-butadiene), poly(propyl methacrylate-butadiene), poly(butyl methacrylate-butadiene), poly(methyl acrylate-butadiene), poly(ethyl acrylate-butadiene), poly(propyl acrylate-butadiene), poly(butyl acrylate-butadiene), poly(methyl methacrylate-isoprene), poly(ethyl methacrylate-isoprene), poly(propyl methacrylate-isoprene), poly(butyl methacrylate-isoprene), poly(methyl acrylate-isoprene), poly(ethyl acrylate-isoprene), poly(propyl acrylate-isoprene), poly(butyl acrylate-isoprene), poly(styrene-isoprene), poly(methylstyrene-isoprene), poly(styrene-propyl acrylate), poly(styrene-butyl acrylate), poly(styrene-butadiene-acrylic acid), poly(styrene-butadiene-methacrylic acid), poly(styrene-butadiene-acrylonitrile-acrylic acid), poly(styrene-butyl acrylate-acrylic acid), poly(styrene-butyl acrylate-methacrylic acid), poly(styrene-butyl acrylate-acrylonitrile), and poly(styrene-butyl acrylate-acrylonitrile-acrylic acid).

5. The recording media of claim 1 wherein said media further comprises a primary coating layer on a back side of the raw base substrate.

6. The recording media of claim 1 wherein said media further comprises an adhesive layer on a back side of the raw base substrate.

7. The recording media of claim 6 wherein the adhesive layer includes a partially esterified polyvinyl alcohol (PVA) or a chemical modified starch.

23

8. The recording media of claim 1 wherein a difference of solubility parameters between the latex component of the ink composition and the polymeric adhesion promoter of the recording media is less than 0.8 (cal·cm<sup>-3</sup>)<sup>1/2</sup>.

9. A recording media, comprising:

a raw base substrate having an image side;  
 a primary coating layer disposed on the image side;  
 a top image receiving layer disposed on the primary coating layer, the image receiving layer comprising a polymeric adhesion promoter formed from an aqueous emulsion having a minimum film forming temperature (MFFT) at, or not less, than 80° C., and including latex particles having a particle size from about 150 to about 350 nanometers, the latex particles having a glass transition temperature at, or above, 90° C.; and  
 an ink composition disposed on the top image receiving layer, the ink composition comprising a latex component;  
 wherein the latex component of the ink composition is identical to the polymeric adhesion promoter present in the image receiving layer of the recording media.

10. The recording media of claim 1 wherein the raw base substrate is a cellulose paper base.

11. A method of making the recording media of claim 1, the method comprising:

a. applying the primary coating layer on the image side of the raw base substrate;  
 b. drying the primary coating layer;  
 c. applying the top image receiving layer over said primary coating layer, wherein said image receiving

24

layer comprises an inorganic pigment filler, a polymeric binder, and the polymeric adhesion promoter;  
 d. jetting the ink composition containing the latex particles onto said top image receiving layer, to form a printed image.

5 12. The method of claim 11, further comprising drying the printed image.

13. The method of claim 11 wherein the primary coating layer is applied on the image side and on a back side of the 10 raw base of the media.

14. The method of claim 11 wherein an adhesive layer is applied on a back side of the raw base substrate.

15. The printing method of claim 11 wherein a difference of solubility parameters between the latex component of the 15 ink composition and the polymeric adhesion promoter of the recording media is less than 0.8 (cal·cm<sup>-3</sup>)<sup>1/2</sup>.

16. A printed article comprising the recording media of 20 claim 1, on which a printed feature has been formed with the ink composition, wherein:

the latex component of the ink composition has a glass transition temperature that is at, or above, 90° C.

17. The printed article of claim 16 wherein a difference of 25 solubility parameters between the latex component of the ink composition and the polymeric adhesion promoter of the recording media is less than 0.5 (cal·cm<sup>-3</sup>)<sup>1/2</sup>.

18. The printed article of claim 16 wherein the latex component of the ink composition is identical to the polymeric adhesion promoter present in the image receiving layer of the recording media.

\* \* \* \* \*